

## UNITED STATES PATENT OFFICE

2,132,579

METHOD FOR PRODUCING UNHAIR ED  
HIDES WITH THE AID OF MOLD TRYPTASES

Otto Röhm, Darmstadt, Germany

No Drawing. Application March 25, 1936, Serial  
No. 70,890. In Germany April 2, 1935

6 Claims. (Cl. 195—6)

The invention relates to preparing hides or skins for tanning, and more particularly to subjecting such hides or skins for depilating and/or bating purposes to neutral or weakly acid solutions containing mold tryptase, particularly those produced by the *Aspergillus* varieties, in the presence of sodium bisulphite.

It is known to bathe and dehair skins and hides with the aid of pancreatic enzymes, particularly the tryptases.

In the bathing process, ammonium salts are generally used along with the enzymes; due to the action of the lime content of the hides, these produce ammonia.

15 In the depilatory process, sodium bicarbonate is largely used which, on reaction with the caustic soda content of the hide, is transformed into sodium carbonate.

Hence, in one case ammoniacal and in the other case soda-containing hides are obtained. This condition of the hides has the drawback that when these hides encounter calcium bicarbonate or calcium sulphate or water containing both, insoluble calcium carbonate is formed which settles out mainly on the grain of the hide and subsequently deleteriously affects the dyeing capacity of the leather. A further drawback resides in the fact that the so-called basic hairs are sometimes difficult to remove.

30 Various attempts have been made to replace the pancreatic tryptase by mold tryptases and to operate in alkaline, acid, or even neutral solutions. But in using mold tryptases difficulty has always been experienced in removing the base and basic hairs.

35 It has been found that all of the aforesaid drawbacks may be obviated when mold tryptases, particularly those produced by the *Aspergillus* varieties, of which *Aspergillus flavus* is an example, are used in neutral to weakly acid solutions together with sodium bisulphite. By this procedure clean hides completely free from basic hairs have been obtained to an extent not entirely achievable hitherto. This procedure also requires that the use of alkali be reduced to about half.

40 It has further been found that the action of the solution used in accordance with the invention may be further improved by the addition of ammonium salts, e. g. ammonium sulphate.

## Examples

1. 100 kgs. of calf hides, softened as usual, are treated with 500 liters water, 1.8 kgs. caustic soda, 45 1.2 kgs. sodium sulphate. After two to three days

the hides are placed in the dehairing bath with 500 liters water of 25° C., 3 kgs. sodium bisulphite, 5 kgs. common salt, and 1 kg. mold tryptase. After one day the hides are obtained in a depilated condition, free from basic hairs. The hides 5 may then be worked up without subsequent bathing.

2. 100 kgs. calf hides, softened as usual, are treated with 500 liters water, 1.8 kgs. caustic soda, and 1.2 kgs. sodium sulphate. After two to three 10 days the hides are placed in the depilating bath with 500 liters water at 25° C., 2.3 kgs. sodium bisulphite, 1.5 kgs. ammonium sulphate and 1 kg. mold tryptase. After one day they are depilated free from basic hair. The hides may then be 15 worked up as usual without subsequent bathing.

3. Ordinary lamb hides treated with lime-arsenic are (after the wool is removed) washed for two hours with soft water and then each 100 kg. weight of hide is bathed with 300 liters water 20 at 25-30° C., 2 kgs. sodium bisulphite, 1 kg. ammonium sulphate and .35 kg. mold tryptase. The bathing may be carried on over night. The next morning the hides are worked up as usual, that is, de-fleshed, smoothed, washed and finished. 25

## I claim:

1. A method of preparing hides or skins for tanning, which comprises pre-treating the hides with an alkaline reagent and then subjecting the pre-treated hides or skins for depilating and bating purposes to a neutral to weakly acid solution containing a mold tryptase together with sodium bisulphite.

2. A method of preparing hides or skins for tanning, which comprises pre-treating the hides 35 with an alkaline reagent and then subjecting the pre-treated hides or skins for depilating and bating purposes to a neutral to weakly acid solution containing a mold tryptase together with sodium bisulphite and an ammonium salt.

3. A method of preparing hides or skins for tanning, which comprises pre-treating the hides with an alkaline reagent and then subjecting the pre-treated hides or skins for depilating and bating purposes to a neutral to weakly acid solution 45 containing a mold tryptase together with sodium bisulphite and ammonium sulphate.

4. A method of preparing hides or skins for tanning, which comprises pre-treating the hides with an alkaline reagent and then subjecting the pre-treated hides or skins for depilating and bating purposes to a neutral to weakly acid solution 50 containing a mold tryptase together with sodium bisulphite, the tryptase being derived from *Aspergillus* varieties.

5. A method of preparing hides or skins for tanning, which comprises pre-treating the hides with an alkaline reagent and then subjecting the pre-treated hides or skins for depilating and bating purposes to a neutral to weakly acid solution containing a mold tryptase together with sodium bisulphite, the tryptase being derived from *Aspergillus flavus*.
6. In a process for preparing hides or skins for

tanning which includes the steps of pre-treating the hides with an alkaline reagent and then subjecting the pre-treated hides for depilating or bating to a solution containing a mold tryptase; the improvement which consists in carrying out the depilating and bating treatment with the tryptase in a neutral to weakly acid solution in the presence of sodium bisulphite. 5

OTTO RÖHM.